

# UNITED STATES PATENT OFFICE.

ALVAH W. CLEMENT, OF CLEVELAND, OHIO, ASSIGNOR TO THE CLEVELAND BRASS  
MANUFACTURING COMPANY, OF CLEVELAND, OHIO, A CORPORATION OF OHIO.

## ALLOY.

1,375,082.

Specification of Letters Patent. Patented Apr. 19, 1921.

No Drawing.

Application filed August 15, 1918. Serial No. 249,950.

To all whom it may concern:

Be it known that I, ALVAH W. CLEMENT, a citizen of the United States, residing at Cleveland, in the county of Cuyahoga and 5 State of Ohio, have invented a certain new and useful Improvement in Alloys, of which the following is a full, clear, and exact description.

The purpose and object of the invention 10 about to be described is the production of an alloy which shall embody qualities that make the alloy highly desirable for use in the fabrication of articles that may be used in the handling of corrosive liquids such as 15 acids, and which shall at the same time possess physical properties which permit it to be easily worked, machined, and otherwise manipulated in the fabrication of articles by tools and methods which are at 20 present employed in working metals.

The proposed alloy further possesses 25 properties which make it valuable for use as an electrical resistance element, the alloy being high in its specific resistance, at the same time possessing the physical properties 30 of ductility and malleability which permits of its being rolled into sheets or drawn into wire form.

Generally speaking, the invention 35 comprises the elements set forth in the accompanying claims.

The alloy herein proposed, in its broadest 40 aspect comprises an alloy of nickel and molybdenum. Both of these elements in 45 their metallic state have acid resisting properties, and when they are combined in the form of an alloy the resisting properties are enhanced.

The proportions of nickel and molybde- 45 num which may be used for the purpose, may be varied through a wide range, but because of the high price of metallic molybdenum, or the source from which molybdenum may be obtained for alloying purposes, 50 it is desirable to use in the alloy as high a percentage of nickel as possible without sacrificing the desired qualities in the alloy.

An alloy consisting of substantially 90% 55 of nickel and substantially 10 per cent. of molybdenum is the best alloy for the purpose desired. However, in view of the fact that molybdenum alloyed with iron is easier 60 and cheaper to obtain than the pure molybdenum, an alloy of 80 per cent. nickel, 10 per cent. molybdenum and 10 per cent. iron

will produce very satisfactory results, and forms a very efficient and useful alloy for the purposes desired.

In the making of the alloy, it is desirable, however, to utilize certain other elements for 60 properties which they impart to the alloy, and for this reason I have found it desirable to use silicon in the proportion of the alloy to such an extent as will appear in the final 65 alloy, from  $\frac{1}{4}$  to  $\frac{1}{2}$  of 1 per cent.

I also find it advisable to use some manganese, this being small however, not less than substantially  $\frac{1}{10}$  of 1% but not exceeding  $\frac{3}{10}$  of 1 per cent.

The silicon increases the fluidity of the 70 alloy thereby increasing the ease with which it may be handled during the pouring. The manganese tends to increase the tensile strength. The manganese, however, must be kept low in order not to counteract other 75 desirable qualities in the alloy, to wit, malleability and ductility.

It is desirable to add to the alloy at the 80 time the nickel is melting, a very small amount of magnesium, less than 1 per cent., the amount of magnesium being so small that it does not appear in an analysis of the final alloy. The small amount of magnesium thus added, imparts to the final alloy, 85 physical properties which enhance its workability, such as wiring and drawing.

It may be desirable also, to add a very 90 small quantity of vanadium to act as a scavenger, to clear the structure and give a good grain to the alloy.

In using silicon and manganese, or any of 95 the other elements mentioned, the amount of nickel and molybdenum in the final alloy will be kept as high as possible, the other elements being added at the expense of the iron.

The alloy which has been described, possesses the physical properties of ductility, high tensile strength, and is easily machinable. The alloy is resistant to corrosive 100 liquids such as certain acids, particularly cold dilute sulfuric, nitric and hydrochloric acids. It is also resistant to corrosion with respect to hot dilute sulfuric acid up to approximately 200° Fahrenheit.

In the alloy which has been discussed 105 above, cobalt may be used in place of nickel, and in the case of articles which may be made to use in connection with the handling of dilute hydrochloric acid, an alloy as 110

above specified, in which cobalt is substituted for the nickel, is preferable.

Because of the machinability and other physical properties which have been mentioned, together with its resistance to corrosion by acids, such an alloy is highly advantageous for use in the manufacture of containers, pipes, cocks, pumps, and other articles which go to make up equipment for handling acids as before specified.

In fact, the alloy is of general use for the fabrication of any article where the property of resistance to corrosion of the dilute acids before mentioned is to be overcome.

An alloy of nickel and molybdenum, or cobalt and molybdenum possesses certain properties which make it highly useful to be used as an electrical resistance material. The ductility of the alloy permits its readily being rolled into sheets or drawn into wire, which are physical properties necessary in making electrical resistance material.

Furthermore, the alloy has high specific resistance which makes it a good resistance element for heating purposes. An alloy of molybdenum with nickel or cobalt and iron in the proportions which have heretofore been mentioned, may also be advantageously used as an electrical resistance element.

In the use of the alloy in this connection, the amount of manganese utilized would be slightly higher than that which has heretofore been specified.

In an alloy of nickel and molybdenum, manganese to the extent of 3 or 4 per cent. might be used. In fact, manganese could be used to as great an extent as possible, up to the point where it would affect the malleability and ductility of the final alloy.

In the event that an alloy of nickel or molybdenum and iron is used, the amount of manganese which could be employed would be less, probably from 1 $\frac{1}{2}$  to 2 per cent.

An alloy of nickel and molybdenum or nickel, molybdenum and iron with manganese for electrical resistance purposes, would be prepared by the addition of small amounts of magnesium or aluminum to the metal when in melted condition, the addition of magnesium increasing the workability, that is to say, the properties of easy rolling and drawing, and both elements being easily oxidizable form a protecting film of oxid, thus preventing further oxidization of the alloy.

In using the alloys for electrical resistance purposes, the silicon employed might be slightly higher than that which was mentioned in the earlier part of the specification.

The silicon not only increases the resistance, but also assists in preventing oxidization of the alloy when used as an electrical resistance element.

The foregoing alloys of molybdenum and nickel, or cobalt, and of molybdenum, iron

and nickel, or cobalt, being subject to oxidization at moderate temperatures, which oxides are largely composed of molybdenum oxid. This oxid forms a resistant coating and I have found that the alloy is available for use for making or lining vessels or pots in which brass, bronze, or forms of ferrous metals are heated.

The alloy is not attacked or affected by lead, zinc, copper or tin, and thus these elements or combinations of them may be melted or handled while in heated melted state in vessels composed of the alloys herein proposed without corrosion of the vessel.

Doubtless other uses may be found for the alloy herein described, which result from the peculiar and particular properties inherent in the alloy.

Inasmuch as nickel and cobalt in the alloy herein described have substantially the same properties, it is to be understood that nickel and cobalt are interchangeable in the alloy, and therefore in the claims where there is mentioned "a metal having the properties of nickel and cobalt" it is intended to include by that expression, either nickel or cobalt.

Having described my invention I claim:

1. An alloy containing as its principal ingredients molybdenum and a metal having the properties of nickel and cobalt together with an appreciable amount of manganese, the manganese being present in amounts not greater than 4%.

2. An alloy containing as its principal ingredients molybdenum and a metal having the properties of nickel and cobalt together with an element having the properties of manganese.

3. An alloy containing as its principal ingredients molybdenum, in amount not greater than 10 per cent., a metal having the properties of nickel and cobalt in amount not greater than 90 per cent. and a metal having the properties of manganese in amount not less than substantially  $\frac{1}{10}$  of 1% but not greater than 4 per cent.

4. An alloy containing as its principal ingredients molybdenum, in amount not greater than 10 per cent., a metal having the properties of nickel and cobalt in amount from 80 to 90 per cent. and a metal having the properties of manganese in amount not less than substantially  $\frac{1}{10}$  of 1% but not greater than 4 per cent.

5. An alloy containing substantially 80 per cent. of a metal having the properties of nickel and cobalt, substantially 10 per cent. of molybdenum, substantially  $\frac{1}{10}$ th per cent. to 4 per cent. of manganese, the remainder of iron.

In testimony whereof, I hereunto affix my signature.

ALVAH W. CLEMENT.